

Nov. 3, 1925.

1,560,450

R. M. WESELY

ARTIFICIAL STONE AND PROCESS OF MAKING

Filed June 15, 1925

*Fig. 10*



*Fig. 10*



*Fig. 10*



INVENTOR.

RALPH M. WESELY

BY

*Thom & Co.*

ATTORNEYS.

## UNITED STATES PATENT OFFICE.

RALPH M. WESELY, OF LOS ANGELES, CALIFORNIA, ASSIGNOR OF ONE-HALF TO  
GEORGE SMITH MACGRUER AND ONE-HALF TO ROBERT MORTON SIMPSON, BOTH  
OF SAN FRANCISCO, CALIFORNIA.

## ARTIFICIAL STONE AND PROCESS OF MAKING.

Application filed June 15, 1925. Serial No. 37,361.

*To all whom it may concern:*

Be it known that I, RALPH M. WESELY, a citizen of Czechoslovakia, and a resident of Los Angeles, in the county of Los Angeles 5 and State of California, have invented a new and useful Artificial Stone and Process of Making, of which the following is a specification.

My invention relates to artificial lava or 10 other stone and a new and novel process of manufacturing same.

My invention is more particularly directed to artificial stone having those characterizing features which cause the finished 15 product to very closely and in fact minutely compare with natural travertin, particularly Roman travertin, often called "travertin marble", the natural being the calcareous deposit from springs in many localities of Italy and sometimes quarried in some parts of the United States of America. This natural marble or stone is characterized by a striated or veined surface, the veining 20 being of slightly different color from the body of the marble. This striated or veined surface is arranged relatively but in no true or consistent order of the arrangement of 25 serrated voids which appear in the natural travertin mostly on the surface thereof. 30 These voids appear undercut, and it would seem to the eye that they extend clear through the stone, presenting the appearance of aged worm eaten material. The natural, as well as the artificial travertin, is 35 used for decorative interior and exterior purposes in building construction and it is customary that same be in the form of relatively thin slabs. The material is not only decorative but same is very desirable 40 because of its properties for absorbing sound, the porous like qualities serving to break up sound waves and reduce reflection very materially.

It is not broadly new in the art to produce 45 what is called imitation travertin, but, to the best of my knowledge, all attempts have fallen short when the results and characteristics of these imitations are compared with a specimen of natural sedimentary origin. 50 In these imitations provided heretofore, sur-

faces characterized by color striation and voids have been produced, but in each has been absent certain characteristics of the natural marble, namely, many voids of almost minute or consistent size appearing 55 promiscuously upon the surface of the material. These minute or pin holes, so to speak, appear school like or stippled, and are generally apart from the separated voids aforementioned, the latter being of irregular 60 sizes as against the consistency in size of these so-called pin holes.

Aside from other niceties of arrangement and order of the parts forming my invention, it is particularly an object of my invention to produce these pin holes and arrange same promiscuously upon the surface of the finished product in near natural like order with the larger voids and the differently colored veins or striations. By producing the minute or pin holes or voids in the material, I not only am able to produce an almost exact duplicate of the natural stone and thereby enhance the value of the material architecturally in view of its attractive and ornamental appearance, but I augment the acoustical properties of said material.

Aside from the improvements above pointed out which give to the finished product the elegance and beauty of the natural stone and one which follows the rhythmical order of the veining and all voids, I have carried into actual practice, a method or process of producing imitation travertin which is simple, inexpensive and capable of being carried on to produce material in great quantities with maximum rapidity and with consistency.

In the article which results from the practice of my invention, I have produced one which is strong and durable and of light weight.

With the above and other objects in view which will appear as the nature of the invention is better understood, the same consists in the improved construction and novel arrangements of parts which will herein-after be fully described and particularly pointed out in the claims.

In the accompanying drawings has been illustrated a single and preferred form of the invention, it being, however, understood that no limitations are necessarily made to the precise structural details therein exhibited, but that changes, alterations and modifications within the scope of the claims may be resorted to when desired.

Figure 1 is a plan view of a mold showing 10 the manner of carrying the first step of the process into practice;

Figure 2 is a plan view of a slab of material produced by my process; and

Figure 3 is a section on line III—III of 15 Figure 2.

I shall first proceed to describe the article or imitation stone produced by following the steps and employing the materials and compositions of matter which constitute the 20 novel features of my invention, and for this purpose, reference may be best had to Figure 2 of the drawings forming part of this specification.

The slab A is formed of plastery or cementitious material cast from a mold of suitable well known form or otherwise produced, following the choice or skill of the artisan. This slab is characterized by a surface having veins or striations B of suitable 25 color tone and of a slightly different color from the body of the slab. Between the veins or striations B and extending to the outer surface of the slab are voids C which appear undercut and serrated, giving to the 30 eye the effect that certain of them extend clear through the slab. These voids C are of irregular shapes and sizes throughout the outer surface of the slab and same appear rather promiscuously, and are sometimes 35 isolated with respect to each other, while, at other times or places upon the slab, groups of these voids come into almost and frequently are in conjoined relation. I want to 40 clearly distinguish the voids C from other 45 voids or surface inconsistencies and for this reason, shall subsequently refer to them as large voids, and they may be bounded as such by the dot and dash lines shown in Figure 2. These undercut large voids are of 50 dark color at their closed ends to produce the desired shadow effect.

The veins or striations are irregularly shaped and sometimes in casting or working the materials, small or varying sized 55 splotches of this vein material of one color will be found imbedded in vein material of a different color as indicated at D.

To this point, except for some few but important changes, this description or outline 60 of the characterizing features of my artificial stone agrees with some of the features which characterize prior known imitations of travertin, the difference in my new method of producing the material notwithstanding. By this, I mean to say that the

character of the ornamental surface of the slab is to a large extent similar, but the qualities of my slab are quite different, and also is it true that I have produced an imitation which patterns more closely after the 70 natural travertin.

Now, it will be observed that at points appearing promiscuously upon the slab are small voids or pin holes E. It is these holes that characterize a large part of the natural 75 stone and without them, the prior attempts to reproduce the natural have failed. These small voids or pin holes run in schools or groups in varying but greatly multiplied number in comparison with the number of 80 voids C. Sometimes, these small voids will be found side by side with the large voids, and in other places upon the finished slab, these small voids will appear in entirely separated groups. The large voids are distinguished for the purpose of clearness from the small voids by the dotted lines F in Figure 2, and it will be observed that said 85 small voids are shallow and that in the cross section through the slab as illustrated in 90 Figure 3, they run through portions of the thickness of the slab and are stratified relatively; parts of the slab being sponge-like. In other words, they are in substantially conjoined relation through parts of the 95 slab's thickness and they are similarly in conjoined relation on the outer surface of the slab.

I have now made general reference to the 100 characterizing features of my finished article which cause it to truly correspond with the natural travertin. By changing the porosity of the material through its thickness as provided for by the small holes or voids E, added acoustic properties are grafted into 105 the material as contributory to the sound deadening properties of the large voids, and, at the same time, I have injected into the material those features which result in a true simulation of the natural travertin to 110 the eye of the most able critic.

#### *Body mix and veining.*

As a plastery body, I may employ any 115 suitable well known materials, such as (1) plaster of Paris or (2) Keene's cement or (3) Portland cement. In either event, the material is mixed with water until the desired consistency is had. I then take suitable parts of this plastery material and add 120 coloring matter thereto until the desired tone, generally soft gray, is obtained. Portions of the body mix and portions of the colored subdivided parts thereof are now poured or otherwise suitable deposited upon a previously prepared mold surface, as shown at A', (Figure 1) so as to form the veins or narrow layers B. By previously prepared mold, I of course refer to the customary greased surface onto which the ma- 130

terial to be cast is deposited. When this is accomplished, a comb, brush or the like can be run over the veins to make same appear irregular with the veins of one color tone sometimes running into veins of another color tone.

*Large under cut voids.*

I then take a suitable batch or quantity of the body mix and incorporate it with bicarbonate of soda, tartaric acid, marble dust and coloring matter. To this, I add a suitable quantity of alcohol. These parts are thoroughly mixed together at a proper consistency and worked to finally produce particles or dry, effervescent, partly soluble lumps of small bits of varying sizes. These particles are now sprinkled upon the exposed surfaces of the mold between the veins so as to produce many large voids upon the exposed surfaces of the material while these lumps are in a dry void forming state. When subjected to the action of a stream of water after the mass has set, the lumps are broken down and can be readily washed out, except for some particles, which remain upon the walls of the formed voids. These particles act to darken the color of the walls so as to produce an aged effect. It shall be understood that the undercut voids are formed by the lumpy particles while the latter are in a dry state and not by any chemical action that would tend to ream or bore these voids.

*Small voids.*

I now take a batch of the previously prepared body mix and add an effervescent agent thereto and to give body and to assist the action of the agent, I preferably add a suitable part of marble dust or rice flour. This effervescent agent may be in the form of (1) sulphuric, or (2) muriatic acid, or (3) alum water or the like. I gauge my mixtures in this instance so that bombardment of the plastery mix will take place through effervescence of the chemicals employed to form small pin holes in that part of the mix in which this chemical incorporation exists. This batch is then splashed, poured, spread or otherwise placed over the veins and around places occupied by the lumpy particles. If desired, the lumpy material may be arranged on the mold first and the veining material placed over and around same.

*Backing.*

The remainder of the body mix or a mass of plastery matter of suitable color tone is then spread over the portions treated as now set forth and the material permitted to set and harden.

With further reference to the step of pro-

ducing the large undercut voids, the chemicals employed may be in the following proportions:—

|                           | Parts. |
|---------------------------|--------|
| Tartaric acid             | 10 70  |
| Sodium bicarbonate        | 9      |
| Marble dust or rice flour | 6      |
| Alcohol suitable amount.  |        |

For the small voids I may use the following proportion of chemicals:—

Sulphuric acid, 1 part to 50 parts water; or muriatic acid, 1 part to 25 parts water; or alum water, 1 part to 3 parts water, and suitable quantity of rice flour or marble dust.

After the cast material has set and dried, same may be subjected to the action of a stream of water so that the latter will come in physical contact with the dry lumpy particles which go to make the large voids, and same is caused to be evacuated from the slab, leaving charred like undercut serrated voids.

It should be clearly understood that the effervescent agency employed herein shall never function to such violent extent as to form holes or pricks E upon the surface of the finished stone of a size much larger than the smallest hole or void C produced by means of the chemicals recited herein.

It is found that in carrying out my process, gelatin molds can be employed on which the plastery materials are poured and that incident to the fact that no heat is created when the chemicals employed herein function, the mold is maintained in a cool state, and that when the cast slab is removed from the mold, it is in no way distorted, as would be the case were the plastery materials subjected to the action of heat, as in the case where calcium carbide, for example, would be used. Nor do I experience any trouble that in any way injures the mold. The materials used in forming the aforesaid large voids cause these voids to appear as though they had been treated with burnt umber or like matter, giving to the voids the much-sought-for effect not produced herebefore in processes of making imitation lava stone, imitation travertin or the like.

It will do no objection to again emphasize the fact that the loose lumpy particles from which the so-called large undercut voids are formed are active for producing these voids while they are in a dry state and that the form or shape of the void is in agreement with the form or shape of the lumpy particle from which the void is cast.

I claim:

1. Artificial stone consisting of a plastery material at least one surface of which is shaped and striated and formed with sets of undercut voids and additional sets of

- small voids, the striae constituting the exposed portions of shallow inlays of colored plastery material.
2. Artificial stone consisting of a plastery material at least one surface of which is shaped and striated and formed with sets of undercut voids and additional sets of small voids, the striae constituting the exposed portions of shallow inlays of colored plastery material, and the small voids being formed in plastery materials of different porosity through the thickness of the stone than that of the body of the stone at the undercut voids.
3. Artificial stone consisting of independent plastery materials of respectively different degrees of porosity, correlated with striations of respectively different color tone, constituting the exposed portions of shallow inlays, all in simulation of a natural stone of sedimentary origin.
4. As a new article of manufacture, artificial stone characterized by plastery materials of respectively different color tones arranged to produce striations on one face of the stone, the striae constituting the exposed portions of shallow inlays, and provided with irregularly spaced depressions, and other materials providing upon the said one face of the stone groups of small depressions.
5. As a new article of manufacture, artificial stone characterized by plastery materials of respectively different color tones arranged to produce striations on one face of the stone, the striae constituting the exposed portions of shallow inlays, and provided with irregularly spaced undercut depressions, and other materials providing upon the said one face of the stone groups of small depressions.
6. Artificial stone comprising plastery material at least one surface of which is shaped and striated and formed with small irregularly spaced depressions whose walls are charred to give shadow and age effect to the depressions, the striae constituting the exposed portions of shallow inlays of colored plastery material.
7. As a new article of manufacture, artificial stone formed of plastery materials of respectively different color tone presenting inlays of colored striae upon one surface of the stone, and formed with undercut depressions extending onto said surface, and other materials of different properties conjoined with the first named materials, and provided with many small pin holes exposed to said surface of the stone.
8. Artificial stone comprising a striated mass of plastery material provided with irregularly shaped surface voids and relatively consistently formed surface stippling.
9. Artificial stone comprising a striated mass of plastery material provided with irregularly shaped surface voids having charred walls and relatively consistently formed surface stippling.
10. The herein described process of manufacturing striated artificial stone which consists in depositing upon a mold surface a series of narrow layers of plastic material, depositing upon the exposed surfaces therebetween a material of such texture and consistency as will leave numerous portions of said exposed surfaces out of contact with said material, depositing plastic effervesced material upon the mold between some of said layers to produce numerous voids mostly of infinitesimal size upon one surface of the stone, binding said layers and all of said materials together, and allowing the mass to set.
11. The herein described process of manufacturing striated artificial stone which consists in depositing upon a mold surface a series of narrow layers of plastic material, depositing upon the exposed surfaces therebetween a material of such texture and consistency as will leave numerous portions of said exposed surfaces out of contact with said material, depositing plastic effervesced material upon the mold between some of said layers to produce numerous voids mostly of infinitesimal size upon one surface of the stone, binding said layers and all of said materials together, and allowing the mass to set, and then causing the second material to be evacuated from the set mass to leave irregularly shaped and respectively different sizes of undercut voids in said one surface of the stone.
12. The herein described process of manufacturing striated artificial stone which consists in depositing upon a mold surface a series of narrow layers of plastic material, depositing upon the exposed surfaces therebetween a chemically prepared dry material of such texture and consistency as will leave numerous portions of said exposed surfaces out of contact with said material while the material is dry, and which said material is adapted to be disseminated when subjected to the action of water after the stone is dry, depositing plastic effervesced material upon the mold between some of said layers to produce numerous voids mostly of infinitesimal size upon one surface of the stone, binding said layers and all of said materials together, and allowing the mass to set.
13. As a new article of manufacture, artificial stone characterized by a plastic mass having an ornamental surface provided with undercut voids in which the voids are formed by lumpy particles of effervesced matter which, when moistened, after the stone is set causes a residue dust of said matter to line the walls of said voids, thereby giving to said walls an aged and shadow like effect.

70

75

80

85

90

95

100

105

110

115

120

125

130

14. As a new article of manufacture, artificial stone characterized by a plastic mass having an ornamental surface provided with undercut voids in which the voids are formed by lumpy particles of effervesced matter which, when moistened after the stone is set causes a residue dust of said

matter to line the walls of said voids, thereby giving to said walls an aged and shadow like effect, and a material incorporated in said mass to give to the ornamental surface a stippled effect.

RALPH M. WESELY.